

# UNITED STATES PATENT OFFICE.

HEXTALL HARVEY KELSEY, OF LONDON, ENGLAND, ASSIGNOR TO NORMAN  
MALCOLMSON, OF LONDON, ENGLAND.

## DYEING.

1,254,810.

Specification of Letters Patent. Patented Jan. 29, 1918.

No Drawing.

Application filed June 4, 1917. Serial No. 172,845.

To all whom it may concern:

Be it known that I, HEXTALL HARVEY KELSEY, a subject of the King of England, residing at London, England, have invented 5 certain new and useful Improvements in Dyeing, of which the following is a specification.

The present invention relates to the employment of sea-weed as a dye-stuff. Pigments of various colors are contained in sea-weed of the melanosperm, rhodosperm and chlorosperm groups. Certain colors are remarkably constant in large natural algae groups. Thus the *Fucaceæ* exhibit a brown or olive color, and the *Florideæ* a beautiful rose-red.

The present invention comprises, subject to the exceptions hereinafter set forth and disclaimed, a process of dyeing by means of 20 a dye-stuff or a dye produced from the melanosperm, rhodosperm and chlorosperm groups of sea-weed.

It is prior knowledge that dulse or duilsg (*Rhodymenia edulis*) has been heretofore 25 used to produce a somewhat fugitive reddish dye and it is to be understood that the use of dulse for the production of reddish dye is not of the present invention and is one of the exceptions above referred to.

30 The inventor has discovered that colors may be imparted to fabrics by merely boiling the particular sea-weed proposed to be used, with the fabric to be dyed; for example from one ounce upward of the weed to a pound of the fabric to be dyed.

The present invention comprises a process 35 of dyeing which consists in putting the material that is to be dyed into a bath of water or spirit containing either in the raw state or in paste or powder form, a sea-weed of the rhodosperm group (except dulse) or the chlorosperm group.

It also comprises a process of dyeing 40 which consists in putting the material that is to be dyed into a bath of water or spirit containing either in the raw state or in paste or powder form, a sea-weed of the melanosperm group, except *Laminaria* in the case when laminaria powder is contained in a 45 paste with indigo according to the specification of expired prior British Letters Patent No. 1789/1902 granted to J. Y. Johnson.

The paste or powder above referred to can be obtained by subjecting the sea-weed to a treatment of boiling in water till it becomes 55 soft and next crushing it so that a paste results, or by roasting the sea-weed and then comminuting the dry weed, much in the same way as coffee and chicory are roasted and ground. The powder may also be obtained by drying a paste such as is above referred to.

When using the paste or powder the color is imparted to the fabric in much less time than when the raw weed is used.

60 The inventor has found that when using the melanosperm or chlorosperm or rhodosperm powder or paste or a dyeing liquid derived from any of these groups of sea-weed the addition to the dye-beck of a sulfuric-acid solution intensifies and deepens the color produced on the fabric. As an example,  $\frac{1}{16}$  of an ounce of powder and  $\frac{1}{16}$  of an ounce of concentrated sulfuric acid 65 mixed with  $\frac{1}{2}$  pint of water will make a 70 good dyeing-liquid.

75 The colors imparted to the fabric from the sea-weed dyes aforesaid are fast colors and do not necessarily involve the use of mordants.

80 All the known dye-stuffs, mordants, liquors, or topping baths may be used, either separately or mixed with the sea-weed, powder or paste or their solutions for the purpose of varying, intensifying or fixing 85 any of the colors if desired.

Different types of weed or the colors obtained therefrom can be mixed, to obtain varying shades and tints.

I am aware that dulse or duilsg (*Rhodymenia edulis*) has been used as a dye and I 90 make no claim to the employment of dulse as a dye-stuff, nor do I claim anything described or claimed in the specification of expired British Letters Patent No. 142/81 95 (Standford) or No. 1789/02 (Johnson).

What I claim as my invention and desire to secure by Letters Patent is:—

1. A process of dyeing by putting the material that is to be dyed into a bath of 100 liquid containing a sea-weed of the melanosperm group.

2. A process of dyeing by putting the material that is to be dyed into a bath of

water containing a sea-weed of the menalosperm group.

3. A process of dyeing by putting the material that is to be dyed into a bath of water containing a sea-weed of the menalosperm group in powder.

4. The addition to a dyeing liquid de-

rived from menalosperm sea-weed of sulfuric acid for the purpose of intensifying or varying the color imparted by the liquid to the material dyed.

In testimony whereof I affix my signature.

HEXTALL HARVEY KELSEY.